

(No Model.)

J. W. MACKNIGHT.  
METHOD OF LAYING ARTIFICIAL PAVEMENT.

No. 401,447.

Patented Apr. 16, 1889.

FIG. 1



FIG. 2



FIG. 3



WITNESSES.

W. C. Lowe  
W. W. Wagner.

INVENTOR

J. W. Macknight  
by his attorneys  
Rector & Bissell

# UNITED STATES PATENT OFFICE.

JOHN W. MACKNIGHT, OF NEW YORK, N. Y.

## METHOD OF LAYING ARTIFICIAL PAVEMENT.

SPECIFICATION forming part of Letters Patent No. 401,447, dated April 16, 1889.

Application filed January 2, 1889. Serial No. 295,197. (No model.)

*To all whom it may concern:*

Be it known that I, JOHN W. MACKNIGHT, of New York city, New York, have invented an Improved Method of Laying Artificial Pavement, of which the following is a specification.

This invention has reference to an improved method of laying an artificial pavement for the roadway between the curbs. It has for its object, more particularly, to produce a noiseless pavement which offers a secure footing for the horses, and in which the yielding material between the artificial-stone strips is securely held in place, and is prevented from being gradually trod into the ground.

In the accompanying drawings, Figure 1 is a vertical transverse section of an artificial pavement laid according to my method. Fig. 2 is a top view of the same, partly in longitudinal section. Fig. 3 is a cross-section through the upper layers on the line  $x x$ , Fig. 1, with the joists in place.

In laying the artificial pavement, I first form a bottom layer of rocks,  $a$ , placed on edge. Above these I form a layer of coal-ashes,  $b$ . These two layers are made to extend over any desired length of the roadway, perhaps a block, from curb to curb. Next I form the third layer of flintic concrete; but this layer I do not form in a continuous section, but in a series of parallel equidistant strips or sections,  $c c$ , extending from curb to curb. The spaces between the sections  $c$  are filled in, in manner hereinafter described, after the top dressing upon sections  $c$  has been completed. Upon the sections  $c$ , I place from curb to curb, while these sections are still moist, a series of joists,  $d d$ , preferably about four inches apart and one inch wide. Near each edge of the sections  $c$ , I place upon it a T-shaped joist,  $d'$ . Next I fill in the spaces between the joists with a wet mixture of trap-rock and Portland cement. Preferably two grades of trap-rock are used—the coarser one for the bottom  $e$  and the finer one for the top  $f$ . The layers  $e f$  are thus composed of the same material, only that the bottom layer is somewhat coarser. The bottom layer,  $e$ , being moist and the flintic con-

crete layer  $c$  being moist, these two layers 50 will unite firmly with each other into one adherent solid mass. The sections  $c$ , with their top layer,  $e f$ , being thus far completed, the end joists,  $d' d'$ , are removed, and the spaces between the sections  $c c$  are filled in 55 in the same manner as has been described with relation to sections  $c$ —that is to say, sections  $c'$  of flintic concrete are formed between sections  $c c$ , and upon them the joists  $d$  are placed. Of course the end joists,  $d'$ , 60 are not needed. Next the two top layers,  $e' f'$ , are filled in between the top layers,  $e f$ , of the adjoining completed sections. It will be seen that owing to the T-shaped end joists,  $d'$ , lap-joints will be formed between the various 65 sections of pavement, which prevent settling along the lines  $g$  of the joints. The pavement being thus far completed, the joists  $d$  are all removed, and the grooves thus formed are filled in with a yielding mixture,  $h$ , composed of about thirty parts of broken trap-rock, gravel, or slag, one part of crude petroleum, and five parts of asphaltum. To form this mixture, the trap-rock, gravel, or slag is first dried, and is mixed with the petroleum and 70 asphaltum while the latter are heated.

The mixture will fill the grooves up to the surface, and will partly percolate through the sides of the grooves into the top layers, to be firmly joined therewith; but, as the top layers 80 are firmly united to the flintic concrete layers  $c c'$ , the bottom of the grooves are solidly closed, and the mixture  $h$  will not be liable to be pressed down and out of the grooves by wear.

Thus a pavement is formed that offers a proper hold for the horses, and which at the same time will last for a very long time.

Another feature of this pavement is that at the lap-joints between the sections of top 90 dressing these sections will not unite—that is, at the lines  $g$  the pavement will be disconnected. Thus any one section may be broken away partly or entirely without disturbing the adjoining sections.

What I claim is—

The method of laying an artificial pavement, which consists in forming continuous

bottom layers of rock and ashes, forming a series of parallel sections of flintic concrete upon them, placing joists upon these sections, filling in the spaces between the joists with a mixture of flintic concrete and cement, removing the end joists and filling in the intervening spaces in a similar manner, remov-

ing the remaining joists, and filling in the grooves with a yielding mixture, substantially as specified.

JOHN W. MACKNIGHT.

Witnesses:

F. V. BRIESEN,  
HENRY E. ROEDER.